

# UNITED STATES PATENT OFFICE.

WILLIAM E. HEDGES, OF POLK BAYOU, ARKANSAS.

## TANNING PROCESS.

SPECIFICATION forming part of Letters Patent No. 447,427, dated March 3, 1891.

Application filed November 28, 1890. Serial No. 372,888. (No specimens.)

*To all whom it may concern:*

Be it known that I, WILLIAM E. HEDGES, a citizen of the United States, residing at Polk Bayou, in the county of Sharp and State of 5 Arkansas, have invented certain new and useful Improvements in Processes of Tanning Hides; and I do declare the following to be a full, clear, and exact description of the invention, such as will enable others skilled in 10 the art to which it appertains to make and use the same.

First. Soak all hides until perfectly soft. Then remove all flesh from the hides. Then lime them with the following composition: 15 twelve gallons of water, ten quarts of lime, and ten quarts of ashes. Immerse the hides in the same. The oftener the hides are aired the quicker the hair will slip. When the hair slips easily, raise the hides and put them 20 in clear water and let them soak a while to prevent the lime from injuring the hands. Then take them to the beam and remove all the hair. Then put them in clear water and let them remain until the lime is all removed. 25 Now take them to the table and with a steel sleek remove all the water possible by working them well on the flesh side. Then they are ready for the tan. Prepare the tan as follows:

30 Second. To sixteen gallons of strong oak ooze, one pound of oak-bark to the gallon of water, add four pounds of salt. Then immerse the hides in the same and let them remain until the grain side has a bright straw 35 color. Then add ten pounds of gum-gambier and sixteen ounces of alum.

Third. Raise the hides three or four times a day for the first day. Then let them remain until tanned, which will take from one 40 to twenty-five days, according to the thickness of the hides. All hides, after being tanned, should be washed thoroughly to remove the ooze and thus prevent staining.

Fourth. Take the hides to the table and 45 with a steel sleek work them thoroughly on the flesh side, and then hang them in the shade. When about half dry, oil on the grain side with tanner's oil and on the flesh side with oil and tallow, in equal parts, and then 50 hang in the shade to dry. When dry, take them to the beam and take a thin shaving off

the flesh side. Now they are ready for blacking.

Fifth. Prepare the blacking as follows: to one quart of oil add ten grains of bicarbonate of potash, two ounces of lamp-black, and one-fourth pint of ooze. Apply the same to the leather with the brush, and when blackened rub well with a woolen rag, and then oil them, and they are finished.

Having described my process, what I claim as new, and desire to secure by Letters Patent, is—

1. The process of tanning hides, which consists in first soaking them until perfectly soft and then removing all flesh; then liming them with the following composition: twelve gallons of water, ten quarts of lime, and ten quarts of ashes; then when the hair slips easily raising them and putting them in clear water to soak a while; then removing all hair; then soaking in clear water until the lime is removed; then removing all water that can be removed by working them on the flesh side; then tanning by immersing them in a mixture of sixteen gallons of strong oak ooze and four pounds of salt and letting them remain until the grain side is a bright straw color; then strengthening the ooze by adding ten pounds of gum-gambier; then adding one ounce of alum to one gallon of ooze; then raising the hides two or three times the first day; then letting them remain until tanned, and then washing thoroughly.

2. The process of tanning hides, which consists in first soaking them until perfectly soft and removing all flesh; then liming them with the following compound: twelve gallons of water, ten quarts of lime, and ten quarts of ashes; then when the hair slips easily raising them and putting them in clear water to soak a while; then removing all hair; then soaking in clear water until the lime is removed; then removing all water that can be removed by working them on the flesh side; then tanning by immersing them in a mixture of sixteen gallons of strong oak ooze and four pounds of salt and letting them remain until the grain side is a bright straw color; then strengthening the ooze by adding ten pounds of gum-gambier; then adding one ounce of alum to one gallon of ooze;

then raising the hides two or three times for  
the first day; then letting them remain until  
tanned; then washing thoroughly; then with  
a steel sleek working thoroughly on flesh side;  
5 then hanging in the shade, and when about  
half dry oiling them on the grain side with  
tanner's oil and on the flesh side with oil and  
tallow, in equal parts; then hanging in the

shade to dry; then taking them to the beam  
and taking a thin shaving off the flesh side. 10

In testimony whereof I affix my signature in  
presence of two witnesses.

WILLIAM E. HEDGES.

Witnesses:

JOHN S. WILKERSON,  
JOSHUA WANN.